

[72] Inventors **Keisuke Shiba;**  
**Masanao Hinata; Reiichi Ohi; Hiroshi**  
**Misu, all of Kanagawa, Japan**  
[21] Appl. No. **680,024**  
[22] Filed **Nov. 2, 1967**  
[45] Patented **Oct. 26, 1971**  
[73] Assignee **Fuji Photo-Film Co., Ltd.**  
**Kanagawa, Japan**  
[32] Priority **Nov. 2, 1966**  
[33] **Japan**  
[31] **41/72263**

[54] **PHOTOGRAPHIC SILVER HALIDE EMULSION**  
**9 Claims, No Drawings**

[52] U.S. Cl. .... **96/130,**  
**96/122**  
[51] Int. Cl. .... **G03c 1/10**  
[50] Field of Search. .... **96/102,**  
**104, 106, 117/34; 260/240.1, 240.65**

[56] **References Cited**  
**UNITED STATES PATENTS**

2,945,762 7/1960 Carroll et al. .... **96/100**

**OTHER REFERENCES**

Cyanine Dyes and Related Compounds, Hamer, page 88,  
 QD401 H25

*Primary Examiner*—William D. Martin  
*Assistant Examiner*—Theodore G. Davis  
*Attorney*—Sughrue, Rothwell, Mion, Zinn & MacPeak

**ABSTRACT:** A photographic silver halide emulsion having incorporated therein the sensitizing dye represented by the following general Formula I:



wherein  $Z_1$  represents the nonmetallic atoms necessary for forming 4-quinoline nucleus,

$Z_2$  represents the nonmetallic atoms necessary for forming a 5- or 6-membered ring,

$R_1$  and  $R_2$  represent substituted or nonsubstituted alkyl groups,

$X$  is an acid anion group,

$m$  is 1 or 2, and

$p$  is 1 or 2, said dye forming an intramolecular salt when  $p$  is 1, and together with a compound having triazine nuclei or pyrimidine nuclei represented by the following general formula II:



wherein  $D$  represents a divalent aromatic group combining with each other the pyrimidinylamino groups or triazinylamino groups shown in the above formula,

$R_3$ ,  $R_4$ ,  $R_5$  and  $R_6$  each represents a hydrogen atom, a hydroxyl group, an alkoxy group, a halogen atom, an amino group, an alkyl amino group or a substituted alkylamino group, such as, a hydroxyalkylamino group, a sulfoalkylamino group, a cycloalkylamino group, an arylamino group and a heterocyclic amino residual group, and

$W$  represents  $CH-$  or  $N-$ .

## PHOTOGRAPHIC SILVER HALIDE EMULSION

## BACKGROUND OF THE INVENTION

## 1. Field of the Invention

The present invention relates generally to a spectrally sensitized photographic silver halide emulsion and more particularly to a spectrally sensitized photographic silver halide emulsion in which the formation of photographic fog has been suppressed and the reduction of the spectral sensitivity during long storage has been prevented.

## 2. Description of the Prior Art

It is well known in the production process of photographic silver halide emulsions that by incorporating a certain kind of sensitizing dye in a silver halide emulsion, the light-sensitive wavelength of the silver halide emulsion is extended to a longer wavelength region. This is technically called spectral sensitization. The intensity of the spectral sensitization is influenced not only by the chemical structure of the sensitizing dye, the properties of the emulsion, such as, the composition of the silver halide, the crystal structure of the silver halide, the concentration of silver ions in the emulsion, the pH of the emulsion and the like, but also by the kinds of stabilizers, wetting agents, hardening agents, and couplers present together in the emulsion. In most cases, these compounds incorporated in the silver halide emulsion other than the sensitizing dye are apt to reduce the spectral sensitization. Also, while a sensitizing dye is able to sensitize spectrally the emulsion when added to the emulsion, the addition thereof to the silver halide emulsion is usually accompanied with certain faults such as the formation of fog, the reduction of the property of keeping spectral sensitivity and the like. Therefore, in order to prepare a photographic silver halide light-sensitive element showing less fog and having a good keeping property, it is highly necessary to inhibit the formation of fog caused by the addition of a sensitizing dye and improve the reduction of the spectral sensitivity, which occurs during the long storage. However, the use of a conventional antifogging agent or a stabilizer for improving drawbacks of the emulsion itself, usually results not only in a remarkable reduction in spectral sensitivity, but also in a decrease in the property of keeping spectral sensitization. Therefore, it must be emphasized that the combination of a sensitizing dye with various kinds of additives to improve the property of the emulsion itself should be selective in order to improve the above-mentioned faults in the spectrally sensitized materials.

Therefore, an object of the present invention is to provide a photographic silver halide emulsion which has been spectrally sensitized and in which the formation of fogging by dyes and also the deterioration in the spectrally sensitizing property of the dye, in the course of storage, have been prevented without reducing substantially the spectral sensitivity.

## SUMMARY OF THE INVENTION

The object of this invention can be accomplished according to the present invention by incorporating in a photographic silver halide emulsion the sensitizing dye represented by the following general formula I:



wherein  $Z_1$  represents the nonmetallic atoms necessary for forming 4-quinoline nucleus,

$Z_2$  represents the nonmetallic atoms necessary for forming a 5- or 6-membered ring,

$R_1$  and  $R_2$  represent substituted or nonsubstituted alkyl groups,

$X$  is an acid anion group,

$m$  is 1 or 2, and

$p$  is 1 or 2, said dye forming an intramolecular salt when  $p$  is 1, and together with a compound having triazine nuclei or pyrimidine nuclei represented by the following general Formula II:

II.



wherein  $D$  represents a divalent aromatic group combining with each other the pyrimidinylamino groups or triazinylamino groups shown in the above formula.

$R_3, R_4, R_5$  and  $R_6$  each represents a hydrogen atom, 5 hydroxyl group, an alkoxy group, a halogen atom, an amino group, an alkyl amino group, a substituted alkylamino group, such as, a hydroxyalkylamino group, a sulfoalkylamino group, a cycloalkylamino group, an arylamino group and a heterocyclic amino residual group, and

$W$  represents  $\text{CH}-$  or  $=\text{N}-$

In aforesaid general formula I,  $Z_1$  may be 4-quinoline nuclei having a substituent, such as, a halogen atom, an alkyl group, an alkoxy group and the like.  $Z_2$  is a nonmetallic atomic group necessary for forming a heterocyclic nucleus, such as, a 4-quinoline nucleus, a 2-quinoline nucleus, a naphthothiazole nucleus, a naphselenazole nucleus, a naphthoxazole nucleus, a benzoselenazole nucleus, a benzothiazole nucleus, a benzoxazole nucleus, a thiazole nucleus, an oxazole nucleus, and the like.  $R_1$  and  $R_2$  may be a lower alkyl group, such as, a methyl group, an ethyl group and a propyl group; substituted alkyl group, such as,  $\beta$ -hydroxyethyl group, a  $\beta$ -acetoxyethyl group, an ethylsulfate group; and the like; a carboxylalkyl group or a derivative thereof such as, a carboxyethyl group, a 2-(2-carboxyethoxy)ethyl group and the like; or a sulfoalkyl group and a derivative thereof, such as, a  $\beta$ -sulfoethyl group, a  $\gamma$ -sulfopropyl group, a 2-hydroxy-1-sulfopropyl group, a 3-methoxy-2-(3-sulfopropoxy)propyl group and the like. One structural feature of the sensitizing dye in this invention is that the dye includes at least one quinoline hetero nucleus.

In formula II,  $D$  may be any divalent atomic group which combines the pyrimidinylamino nuclei each other or the triazinylamino nuclei each other in the above-mentioned formula II, such as, a biphenylene group, a phenylene group, a naphthylene group, a stilbene group, a bibenzyl group and the derivatives thereof.

The feature of the compound shown in general formula II is in a point that the compound has the pyrimidinylamino nuclei or the triazinylamino nuclei bridged to each other by the aforesaid atomic group  $D$ .

The sensitizing dye represented by general formula I can sensitize spectrally in a region from a green to red arbitrarily by selecting two heterocyclic nuclei. In particular, the sensitizing dye used in this invention can spectrally sensitize a silver halide emulsion stronger than the case of using a dye having no quinoline nucleus. Even though the sensitizing dye is a trimethine cyanine dye, it can strongly sensitize spectrally a silver halide emulsion even up to the red region which can be attained by using a pentamethine cyanine dye. Also, many of

65 the sensitizing dyes used in the present invention show M-band type spectral sensitization and such spectral distribution is quite suitable to use in a red-sensitive emulsion layer. On the other hand there are faults, such as, fog caused by the dye is easily formed and the spectral sensitivity obtained tends to be lowered in the course of storage. However, when the sensitizing dye shown by general formula I is incorporated in a silver

70 halide emulsion layer along with the compound shown by general formula II having substantially no absorption in a visible region and having a strong absorption in a near ultraviolet region, the formation of fog by the dye can effectively be inhibited and the reduction in spectral sensitivity in the course

of storage can be almost completely prevented without substantially reducing the spectral sensitivity itself. That is, the compound shown by general formula II not only prevents the reduction of the spectrally sensitizing property of such a trimethincyanine dye showing M-band type spectral sensitization but also markedly increase the spectral sensitivity. This means that the compound shown by general formula II shows surely a remarkable super-sensitizing action in this invention. In general, it is known that super-sensitization is apt to occur in the case of J-band type or H-band type trimethine cyanine dye, while it is unfamiliar that the compound shown by general formula II shows such a remarkable super-sensitization with the sensitizing dye of this invention having M-band type spectral distribution, which is one of the important features of this invention. Further, by using the sensitizing dye shown by general formula I, along with the compound shown by general formula II, the color stain formed by the sensitizing dye after photographic processing is reduced and also the harmful action of couplers present therewith on the spectral sensitization is less. These also are features of the invention.

The compound shown by general formula I and the compound shown by general formula II may be incorporated into a silver halide emulsion separately or together as a solution in a water-soluble organic solvent such as, methanol, ethanol, or alkaline methanol, or as an aqueous solution. In general, the amounts of the compounds shown by general formula I and general formula II to be added to a silver halide emulsion may be controlled according to the properties of these compounds, the properties of the emulsion, the kinds of additives to be added to the silver halide emulsion together with the dyes and the like. They may be used in various ratios.

The silver halide used in the silver halide emulsion may be silver iodobromide, silver chlorobromide, silver chloride and the like. Also, the silver halide emulsion of this invention may be prepared in a conventional manner and may be applied to a proper support, such as, a film of a cellulose derivative, a baryta paper and the like.

In the case of incorporating the compounds shown by the aforesaid general formula I and II in combination to a silver halide emulsion, it is particularly effective to apply to a red-sensitive emulsion for color photographic light-sensitive materials.

Typical examples of the sensitizing dyes shown by general formula I and II are shown below, but it should be understood that the sensitizing dye used in this invention is not limited to them only.



5



10



20



25



30



35



50



55



60



65



70



75



5



6



Among the compounds shown by general formula II and used in this invention, the compound wherein W in said formula is  $-N$ , that is, the compound having an *s*-triazine may be prepared by a known method. The compound wherein W is  $-CH=$ , the compound having the pyrimidine nuclei may be prepared by a similar method to the case of preparing compound IIe and compound IIb as shown below.

### PREPARATION OF COMPOUND IIe

To 100 ml. of acetone and 100 ml. of water were added 12.4 g. of sodium 4,4'-diaminostilbene-2,2'-disulfonate and 11.0 g. of 2,4,6-trichloropyrimidine and the mixture was stirred at 55-65° C. While neutralizing hydrochloric acid formed with the advance of the reaction by adding dropwise an aqueous solution of 10 percent sodium carbonate, the reaction mixture was maintained at a state of from neutral to weak acid. After the end of reaction, the reaction produced was cooled by ice to precipitate a crystal, which was recovered by filtration to provide the product.

### PREPARATION OF COMPOUND IIb

A solution of 17.8 g. of compound IIe and 5.7 g. of  $\beta$ -naphthylamine in 100 ml. of dimethyl formamide was heated for 3-4 hours under refluxing. After cooling, the product was desaltsed by filtration in nitrogen and then neutralized with an aqueous solution of 10 percent sodium carbonate. Thereafter, the unreacted amine was removed by extracting with benzene and the solvent of dimethylformamide and water was removed from the system by distillation under a reduced pressure.

Then, 20 g. of the residue prepared above was heated for 3 hours under refluxing in 100 ml. of aniline and the reaction product mixture was added to about 250 ml. of methanol to precipitate the crystal of the objective compound, which was recovered by filtration and dried.

The present invention will now be explained by referring to the following practical examples.

### EXAMPLE 1.

A methanol solution of  $4 \times 10^{-4}$  mols of the sensitizing dye shown by general formula I was added to 100 g. of a silver iodobromide emulsion prepared by a conventional method, which contains Ag  $\times$  by  $33 \times 10^{-3}$  mols, and furthermore, a methanol solution of  $1 \times 10^{-3}$  mols of the compound shown by general formula II was immediately added in the amount shown in table 1. The emulsion thus prepared was stirred for 1 hour, at 40° C. and then applied to a support in an amount of 7 ml. of emulsion per cabinet size and dried.

Thus prepared light-sensitive material was exposed by an optical wedge through a blue filter passing only light of a wavelength shorter than 500 m $\mu$  and then through a yellow filter passing only light of a wavelength longer than 500 m $\mu$ . The material was then developed for 10 minutes at 20° C. in a black and white developer shown as follows:

### COMPOSITION OF THE DEVELOPER

|                                 |          |
|---------------------------------|----------|
| Methanol                        | 0.3 g.   |
| Potassium metabisulfite         | 1.4 g.   |
| Sodium sulfite (anhydrous)      | 38 g.    |
| Hydroquinone                    | 6 g.     |
| Sodium carbonate (mono-hydrate) | 22.5 g.  |
| Potassium bromide               | 0.9 g.   |
| Citric acid                     | 0.7 g.   |
| Water to make                   | 1,000 ml |

This was followed by fixing. Further, the optical density obtained was measured and the blue sensitivity  $S_b$  and the spectral sensitivity  $S_{opt}$  were measured. The results are shown in table 1.

TABLE 1

| Test No. | Sensitizing dye, ml. |        | Supersensitizer, ml. |     | $S_b$<br>(E) | $S_{opt}$<br>(F) | Fog<br>(G) |
|----------|----------------------|--------|----------------------|-----|--------------|------------------|------------|
|          | (A)                  | (B)    | (C)                  | (D) |              |                  |            |
| 5        | IA                   | 0      |                      |     | 100          | 0                | 0.04       |
|          | IA                   | 1      |                      |     | 95           | 100              | 0.32       |
|          | IA                   | 3      |                      |     | 89           | 130              | 0.60       |
|          | IA                   | 3 IIb  | 4                    |     | 93           | 185              | 0.20       |
| 10       | IB                   | 0      | IIb                  |     | 100          | 0                | 0.04       |
|          | IB                   | 1      | IIb                  |     | 87           | 100              | 0.82       |
|          | IB                   | 3      | IIb                  |     | 103          | 115              | 0.81       |
|          | IB                   | 6      | IIb                  |     | 106          | 105              | 0.91       |
|          | IB                   | 3 IIa  | 2                    |     | 100          | 170              | 0.27       |
|          | IB                   | 3 IIa  | 4                    |     | 100          | 170              | 0.07       |
| 15       | IB                   | 3      | IIb                  | 2   | 100          | 115              | 0.09       |
|          | IB                   | 3      | IIb                  | 4   | 100          | 106              | 0.06       |
| 20       | IB                   | 3 IIc  | 2                    |     | 100          | 132              | 0.63       |
|          | IB                   | 3 IIc  | 4                    |     | 100          | 183              | 0.45       |
| 25       | IB                   | 3 IIId | 2                    |     | 100          | 183              | 0.43       |
|          | IB                   | 3 IIId | 4                    |     | 100          | 115              | 0.35       |
| 30       | IB                   | 3 IIe  | 2                    |     | 100          | 115              | 0.35       |
|          | IB                   | 3 IIe  | 4                    |     | 100          | 183              | 0.40       |
| 35       | IC                   | 0 IIe  |                      |     | 100          | 0                | 0.04       |
|          | IC                   | 1 IIe  |                      |     | 71           | 100              | 0.04       |
|          | IC                   | 3 IIe  |                      |     | 50           | 60               | 0.05       |
|          | IC                   | 6 IIe  |                      |     | 32           | 32               | 0.10       |
|          | IC                   | 3 IIb  | 2                    |     | 80           | 200              | 0.04       |
|          | IC                   | 3 IIb  | 4                    |     | 25           | 115              | 0.04       |
| 40       | ID                   | 0 IIb  |                      |     | 100          | 0                | 0.04       |
|          | ID                   | 1 IIb  |                      |     | 100          | 100              | 0.05       |
|          | ID                   | 3 IIb  |                      |     | 100          | 240              | 0.06       |
|          | ID                   | 6 IIb  |                      |     | 100          | 400              | 0.08       |
|          | ID                   | 3 IIId | 2                    |     | 105          | 280              | 0.05       |
|          | ID                   | 3 IIId | 4                    |     | 98           | 300              | 0.04       |
| 45       | IE                   | 0 IIId |                      |     | 100          | 0                | 0.04       |
|          | IE                   | 1 IIId |                      |     | 100          | 100              | 0.05       |
|          | IE                   | 3 IIId |                      |     | 79           | 166              | 0.08       |
|          | IE                   | 6 IIId |                      |     | 74           | 150              | 0.07       |
|          | IE                   | 3 IIb  | 2                    |     | 79           | 178              | 0.06       |
|          | IE                   | 3 IIb  | 4                    |     | 105          | 316              | 0.06       |

Note: (A)=Sensitizing dye; (B)=Addition amount of the sensitizing dye; (C)=Compound shown by general Formula II; (D)=Addition amount of the compound; (E)=Blue sensitivity  $S_b$ ; (F)=Spectral sensitivity; (G)=Fog.

From the results shown above, it will be clear that by applying the present invention, a photographic silver halide emulsion is produced in which the formation of fog is inhibited without lowering the spectral sensitivity.

### EXAMPLE 2

To 100 g. of a silver chlorobromide emulsion prepared by a conventional method, which contains Ag  $\times$  by  $30 \times 10^{-3}$  mols were added a methanol solution of  $4 \times 10^{-4}$  mols of the sensitizing dye shown by general formula I and a methanol solution of  $1 \times 10^{-3}$  mols of the compound shown by general formula II in the amounts shown in table 2 respectively. The resultant emulsion was stirred for 30 minutes at 40° C. and, with the addition of a hardening agent and a wetting agent, the finished emulsion was applied to a film base and dried. The light-sensitive film thus prepared was placed under a relative humidity of 65-70 percent at 24-30° C., for the long duration shown in table 2 and then the spectral sensitivity  $S_{opt}$  was measured by using such a yellow filter, as in example 1. The results are shown in the following table 2.

TABLE 2

| Test No. | Sensitizing dye, ml. |        | Supersensitizer, ml. |     | (E) | (F) | (G) |
|----------|----------------------|--------|----------------------|-----|-----|-----|-----|
|          | (A)                  | (B)    | (C)                  | (D) |     |     |     |
| 65       | IA                   | 3 IIa  | 0                    |     | 100 | 78  | 63  |
|          | IA                   | 3 IIa  | 2                    |     | 100 | 82  | 82  |
|          | IA                   | 3 IIa  | 4                    |     | 93  | 88  | 83  |
| 70       | IC                   | 3 IIb  | 0                    |     | 100 | 77  | 65  |
|          | IC                   | 3 IIb  | 2                    |     | 222 | 200 | 160 |
|          | IC                   | 3 IIb  | 4                    |     | 208 | 206 | 200 |
| 75       | IE                   | 3 IIId | 0                    |     | 100 | 78  | 63  |
|          | IE                   | 3 IIId | 2                    |     | 110 | 101 | 98  |
|          | IE                   | 3 IIId | 4                    |     | 121 | 120 | 118 |

Note: (A): Sensitizing dye; (B): Addition amount of the sensitizing dye; (C): Compound shown by general formula II; (D): Addition amount of the compound; (E): Relative spectral sensitivity Sopt; (a) Directly after coating; (b) After 1 month; (c) After 4 months.

From the results shown above, it will be clear that by applying the present invention, a photographic silver halide emulsion is produced in which the deterioration of the dye sensitizing property in the course of the storage has been prevented.

What is claimed is:

1. A photographic silver halide emulsion containing at least one sensitizing dye shown by the general formula A:

(A)



wherein  $\text{Z}_1$  represents nonmetallic atoms necessary to form the 4-quinoline nucleus,

$\text{Z}_2$  represents nonmetallic atoms necessary to form a nuclei selected from the group consisting of 5-membered hetero nuclei and 6-membered hetero nuclei,

$\text{R}_1$  and  $\text{R}_2$  each represents a member selected from the group consisting of substituted alkyl groups and a non-substituted alkyl group,

$\text{X}$  represents an acid anionic group,

$m$  is 1 or 2, and

$p$  is 1 or 2, said sensitizing dye forming an intramolecular salt when  $p$  is 1, and

at least one compound shown by the general Formula B;

(B)



wherein  $\text{W}$  represents a member selected from the group consisting of  $=\text{CH}-$  and  $=\text{N}-$ ,

$\text{R}_3$ ,  $\text{R}_4$ ,  $\text{R}_5$  and  $\text{R}_6$  each represents a member selected from the group consisting of a hydrogen atom, a hydroxyl group, a halogen atoms, an amino group, an alkyl amino group, a substituted alkylamino group, an arylamino group, and heterocyclic amino residual group, and

$\text{D}$  represents an aromatic divalent atomic group bonding to each other the pyrimidinylamino nuclei or the traizinylamino nuclei shown in Formula B.

2. The photographic silver halide emulsion according to claim 1 wherein said emulsion is a red-sensitive silver halide emulsion for color photographic light-sensitive elements.

3. The photographic silver halide emulsion as claimed in claim 1 in which the 4-quinoline nucleus completed by  $\text{Z}_1$  has a substituent selected from the group consisting of a halogen atom, an alkyl group and an alkoxy group; and the heterocyclic nucleus completed by  $\text{Z}_2$  is selected from the group consisting of a 4-quinoline nucleus, a 2-quinoline nucleus, a naphthothiazole nucleus, a naphthoselenazole nucleus, a naphthoxazole nucleus, a benzoselenazole nucleus, a benzothiazole nucleus, a benzoxazole nucleus, a thiazole nucleus and an oxazole nucleus; and the aromatic divalent atomic group represented by  $\text{D}$  is selected from the group consisting of



10



4. A photographic silver halide emulsion containing 1,1'-diethyl-4,4'-carbocyanine iodide and at least one compound shown by the formula:



wherein  $\text{W}$ ,  $\text{D}$ ,  $\text{R}_3$ ,  $\text{R}_4$ ,  $\text{R}_5$  and  $\text{R}_6$  have the meanings given in claim 1.

5. A photographic silver halide emulsion containing 1,1'-diethyl-2,4'-carbocyanine iodide and at least one compound shown by the formula:



wherein  $\text{W}$ ,  $\text{D}$ ,  $\text{R}_3$ ,  $\text{R}_4$ ,  $\text{R}_5$  and  $\text{R}_6$  have the meanings given in claim 1.

6. A photographic silver halide emulsion containing 3-(3-carboxypropyl)-1'-ethyl-6,7-benzothia-4'-carbocyanine and at least one compound shown by the formula:



wherein  $\text{W}$ ,  $\text{D}$ ,  $\text{R}_3$ ,  $\text{R}_4$ ,  $\text{R}_5$  and  $\text{R}_6$  have the meanings given in claim 1.

7. A photographic silver halide emulsion containing 3(3-sulfopropyl)-1'-ethyl-8'-methyl-oxa-4'-carbocyanine and at least one compound shown by the formula:



where  $\text{W}$ ,  $\text{D}$ ,  $\text{R}_3$ ,  $\text{R}_4$ ,  $\text{R}_5$  and  $\text{R}_6$  have the meanings given in claim 1.

8. A photographic silver halide emulsion containing 3-(2-hydroxyethyl)-5-chloro-1'-ethyl-thia-4'-carbocyanine bromide and at least one compound shown by the formula:



9. A photographic light sensitive element comprising a support having thereon at least one layer containing a photographic silver halide emulsion as claimed in claim 1.